

May 28, 1935.

W. R. SHIMER ET AL

2,003,094

METAL ARTICLE AND METHOD OF PREPARING SAME

Original Filed Aug. 4, 1930 3 Sheets-Sheet 1



W. R. Shimer  
J. A. Kinney and  
F. O. Kickline.

By R. S. C. Kougherty.  
Attorney

May 28, 1935.

W. R. SHIMER ET AL

2,003,094

METAL ARTICLE AND METHOD OF PREPARING SAME

Original Filed Aug. 4, 1930 3 Sheets-Sheet 2



Fig. 2.

## Inventors

*W. R. Shimer  
J. A. Kinney and  
F. O. Kichline.*

By R. S. C. Vaughan Jr. Attorney

May 28, 1935.

W. R. SHIMER ET AL

2,003,094

METAL ARTICLE AND METHOD OF PREPARING SAME

Original Filed Aug. 4, 1930 3 Sheets-Sheet 3



## UNITED STATES PATENT OFFICE

2,003,094

## METAL ARTICLE AND METHOD OF PREPARING SAME

William Robert Shimer, Bethlehem, and James A. Kinney and Frank O. Kichline, Lebanon, Pa., assignors to Bethlehem Steel Company, a corporation of Pennsylvania

Application August 4, 1930, Serial No. 473,004  
Renewed October 27, 1934

5 Claims. (Cl. 148—12)

Our invention relates to sucker rods and similar articles and methods of preparing same. It also relates to corrosion resisting articles and methods for preparing them. An important purpose is to obtain sucker rods or similar articles which shall have mechanical properties superior to those of the ordinary sucker rod because of subjection to a particular heat treatment. Another object is a sucker rod or other article which shall be relatively incorrodible in service.

Our invention comprises a sucker rod having a normalized structure through the greater portion of its length and having a microstructure in the pin ends resulting from a rapid cooling through the critical range, such metal structure of the pin end merging gradually into the normalized structure of the remainder of the rod. Furthermore, our invention comprises articles, whether sucker rods or other articles, having a surface highly resistant to corrosion producing conditions.

In presenting our invention we shall set forth a specific example of its application but of course it is to be understood that this example is merely illustrative and is not intended to be limiting to the protection which is sought.

In setting forth the invention we shall first briefly state the steps of an illustrative process and the effects produced in a sucker rod and then later we shall set forth somewhat more fully the operation when employing particular equipment.

First, setting forth an outline of the process: A round bar of  $\frac{3}{4}$ " diameter, for example, is rolled in the regular way from steel of the following analysis: Carbon .25 to .80, manganese .50 to .80, nickel .40 to 1.00, and chromium .20 to .55. This is prepared in the desired lengths, say, 25 or 30 feet, for instance, the ends heated in the furnace to a temperature between 2000 and 2250° F. and then subjected to a series of upsetting or forging operations to form a pin end and wrench square. Next the bar is placed in a furnace and is uniformly heated throughout its length to a temperature above the critical range, say from 1550° to 1650° F. This may well take about forty-five minutes. The bar is then removed from the furnace and gripped at its two ends, at the wrench squares, in gripping mechanism, which will later be described. The bar is then placed under tension by exercising a pull on one end against a resistance applied to the other end. The pulling force is suddenly applied so that the condition of tension is initiated with a "snap", thereby effecting a straightening of the rod. At about the same time of placing the rod under tension a cool-

ing fluid is applied to the region at each end which includes the wrench square and the pin end. This application of cooling fluid is continued until these regions of the sucker rod have been rapidly cooled through the critical range. The streams of fluid are discontinued, however, before the greater part of the metal in the remaining regions of the rod has cooled through the critical range. The residual heat in the remaining portion of the rod is utilized to effect a "draw" of the quenched regions. Tension is maintained, in the manner indicated, on the rod until the entire rod passes through the critical range. The rods are now released from the gripping mechanism and allowed to cool upon a cooling table until the temperature has dropped to a temperature of from 600 to 700° F. While at this temperature the rod is immersed in a bath of coke oven tar and then removed therefrom while still at an elevated temperature. The tar bakes or "burns on" to form a firm coating.

Now briefly outlining the effects of this treatment: Rods treated as above outlined have excellent mechanical properties. The grain structure is uniform throughout the greater portion of the rod length merging gradually toward the ends into the structure produced by the quenching operation. There is no sharp line or zone of demarcation between the quenched portions and those portions which were normalized in the air. The pin ends, and those portions adjoining the pin ends, where failure frequently occurs, are uniform in structure and much more resistant to failure than with ordinary rods.

The manner in which the rod is straightened and the maintaining of tension on the rod during the cooling through the critical range avoids the use of any of the ordinary straightening operations which might introduce defects or weaknesses in rod structure.

The treatment with tar in some way changes the condition of the surface of the metal so as to resist corrosion. Apparently, it is not merely due to the protection afforded by the coating of tar baked on the surface, as even beneath the coating the rod surface is resistant to corrosive influences.

Having briefly outlined the process and the effects of such process, we shall now proceed to a more detailed statement of the invention with reference to the apparatus employed. Accordingly, referring to the drawings:

Fig. 1 is a plan view of the equipment used;  
Fig. 2 is an end view looking in the direction of the arrows 2—2 of Fig. 1;

Fig. 3 is a detail longitudinal view of the gripping and quenching mechanism;

Fig. 4 is a cross section of the same mechanism taken on the line 4-4 of Fig. 3; and

5 Fig. 5 is a detail view of the quenching apparatus.

To facilitate an easy understanding of the invention, it may be well to first describe the straightening and tensioning and quenching 10 mechanism.

Device 22 is adapted to grip one end of sucker rod 10 and device 23 the other end. Device 22 is connected by means of chain 24 with cross head 25 mounted on piston 26' of air cylinder 26.

15 Device 23 is connected by means of chain 27 and swivel 27' to cross head 28 to which is attached cable 29 passing over pulley 30 and connected to weight 31.

Devices 22 and 23 are essentially the same in 20 structure; therefore a description of one of them will suffice for both. Arms 32 have rod gripping fingers 33. These arms are provided at an intermediate region with lugs 34 which contain openings 35 whereby the arms may be pivotally 25 mounted in opposing relationship on pin 36, which latter is mounted in the inwardly projecting lugs 37 of supporting body 38. Pivoted to the outer ends of arms 32 are links 39, which latter are pivotally connected to clevis 40. To 30 clevis 40 of device 22 is attached one end of chain 24 and to a corresponding clevis of device 23 is attached an end of chain 27. By means of compression spring 41, placed between arms 32 and held in position by rod 42, arms 32 normally tend 35 to effect a gripping action on the rod by gripping fingers 33.

Supporting bodies 38, which support devices 22 and 23, are provided with circular flanges or tires 43, which rest upon smooth plates 44. Webs 40 45 of bodies 38 are provided with circular holes through which pass nozzles 48 of the end quenching mechanism.

Each of the quenching devices comprises a 45 manifold 46 which is connected with a source of compressed air by means of pipe 47. Connected with manifold 46 are nozzle pipes 48 which are adapted to pass through the holes in web 45. Pipes 48 are provided with openings 49 disposed in proximity to the end regions of the sucker rod, 50 whereby air may be streamed upon wrench square 13 and pin ends 12 of the sucker rod.

Now proceeding to a description of the complete process: The sucker rod 10 having pin end 11, wrench square 12 and with the thickened portion 13 between the wrench square and the shank proper of the rod and collar 14 between the wrench square and the pin end 11, is rolled 55 from the stock stand 15 into charging trough 16. This trough is mounted upon trolleys 16' adapted 60 to roll upon trackways 17. The trough is moved into position opposite grooves 19 of heating furnace 18 and the rod pushed from the charging trough into the furnace. Here the rod is heated for a period of about forty-five minutes to give 65 it a temperature of from say 1550 to 1650° F., substantially uniform from end to end of the rod. Drawing trough 20, mounted upon trolleys 20' and rolling upon trackways 17, is moved into position opposite the rod in furnace 18 and the 70 rod drawn into the trough. The trough is then moved to table 21.

Devices 22 and 23 are now brought into position at the ends of the rod, and arms 32 are pressed together against the action of spring 41 to open 75 the gripping elements 33 and these are placed

in position upon the wrench square 12 at each end of the rod, the pressure of spring 41 serving to effect a gripping engagement of fingers 33 upon the rod. Air is admitted to cylinder 26 and cross head 25 is carried suddenly to the right, as viewed in Figs. 1 and 3, jerking the rod in the same direction and elevating the weight 31. This jerking action is very important as it serves very effectively to eliminate any kinks or other conditions tending to prevent straightness in the rod. At the same time the rod is placed under a substantial tension. For a rod of cross section such as in the present example and of the particular composition and with the particular temperatures involved, about 1000 lbs. has been found suitable for weight 31.

The placing of the apparatus and rod under tension as just outlined, serves to actuate the toggles containing links 39 to produce an effective gripping of fingers 33 upon the ends of the 20 rod.

The motion of cross head 25 serves to operate contactor 51 which closes the circuit through solenoid 51' and thereby serves to open air valve 52 to admit air to manifold 46 and thus to produce a flow of air through openings 49 of nozzle pipes 48 to effect a rapid cooling of the end regions of the sucker rods including pin end 12, wrench square 13 and collar 14. The air flow continues until timer mechanism 53 in the same circuit 30 opens the circuit through solenoid thereby causing valve 52 to close. The time of the quenching operation will vary somewhat but should be sufficient to permit practically the entire mass of the end regions which are receiving the flow of air to cool below the critical range. Following the quenching operation the principal mass of the rod is still above the critical range and the residual heat in the rod serves to effect a "draw" 35 of the quenched metal of the ends.

Tension is maintained on the rod until the entire mass thereof has passed through the critical range. When the rod has cooled below the critical range the gripping mechanisms are 40 released from the ends of the rod which is allowed to cool to a somewhat lower temperature on table 21.

The rod is not completely cooled on table 21 but while still at an elevated temperature, say at a 45 temperature of from 600 to 700° F., the rod is moved therefrom into dipping rack 54 wherein the rod is dipped into a bath of tar 55 and then raised therefrom while still at an elevated temperature to permit the tar to "burn on". The 50 rod is then discharged onto stand 56.

Following the treatment just outlined the pin 55 ends are machine turned and threaded.

Sucker rods thus treated have certain characteristics which especially fit them for the particular type of environment in which sucker rods are used. The quenched end and normalized rod structures, merging gradually into each other, give to the rods just the qualities which enable them most effectively to resist failures in service. The treatment with tar produces a surface which is very resistant to corrosion under conditions where the life of the ordinary rods is frequently seriously curtailed on account of corrosive influences.

Having thus described our invention what we claim and desire to secure by Letters Patent is:

1. In a process of the class described, the steps of upsetting the end of a rod, heating the entire rod above the critical range, subjecting such rod to sufficient tension to straighten, quenching the

end, drawing such quenched end by means of the residual heat in the rod and allowing the rod to cool in the air.

2. In a process for treating articles of the class described, the steps of upsetting the ends, heating the entire rod above the critical range, straightening, cooling the ends rapidly through the critical range, drawing said ends by means of the residual heat in the rod, and allowing the remaining portions of the rod to cool in the air through the critical range to produce a normalized structure.

3. In a process for treating articles of the class described, the steps of upsetting the ends of the rod, heating the entire rod above the critical range, applying sudden tension to straighten the rod, maintaining said rod under tension, quenching the ends of said rod, drawing such quenched ends by means of the residual heat in the rod, and allowing the rod to cool in air through the

critical range to produce a normalized structure in the rod while maintaining tension thereon.

4. A sucker rod of steel containing carbon between .25% and .80%, nickel between .40% and 1.00% and chromium between .20% and .60%, having a normalized structure throughout the greater portion of its length, and having a structure in its pin ends resulting from quenching and drawing, the normalized and quenched and drawn metal structures merging gradually into each other.

5. A sucker rod of steel containing carbon between .25% and .80%, nickel between .40% and 1.00% and chromium between .20% and .60%, having a normalized structure throughout at least the greater portion of its length.

WILLIAM ROBERT SHIMER.  
JAMES A. KINNEY.  
FRANK O. KICHLIN.

**CERTIFICATE OF CORRECTION.**

**Patent No. 2,003,094.**

**May 28, 1935.**

**WILLIAM ROBERT SHIMER, ET AL.**

**It is hereby certified that error appears in the printed specification of the above numbered patent requiring correction as follows: Page 1, first column, line 37, for "55" read .55; and that the said Letters Patent should be read with this correction therein that the same may conform to the record of the case in the Patent Office.**

**Signed and sealed this 9th day of July, A. D. 1935.**

**(Seal)**

**Bryan M. Battey  
Acting Commissioner of Patents.**